

# United States Patent Office

2,742,414

Patented Apr. 17, 1956

1

2,742,414

## ELECTROLYTIC METHOD OF PRODUCING ALUMINUM

Kiichi Itoh, Takarazuka, Japan

No Drawing. Application January 26, 1955,  
Serial No. 484,301

Claims priority, application Japan August 25, 1954

2 Claims. (Cl. 204—67)

The present invention relates to an electrolytic method of producing aluminum and particularly to a method of melting an electrolytic bath at a low temperature in fusing electrolysis of aluminum so that electrolysis is carried out at a low temperature.

The object of the present invention is to provide a method whereby an electrolytic bath is melted at a low temperature in the fusing electrolysis of aluminum, at the same time the solubility of alumina in the electrolytic bath can be increased, the electrolysis temperature can therefore be maintained low, and the damage of the electrolytic cell can be made small.

At the present, most commonly and widely known method of manufacturing aluminum by fusing electrolysis is to add 10 to 15 parts of alumina to 85 to 90 parts of molten cryolite and to electrolyze the fused mixture at a temperature of about 950 to 1000° C. However, keeping the electrolytic bath at such a high temperature has various disadvantages such as acceleration of damage of the cell, difficulty in operation, etc. Therefore, said method is not entirely satisfactory.

I have found that, by using sodium borofluoride and/or aluminum-sodium borofluoride together with cryolite instead of cryolite alone in the conventional method, the solubility of alumina can be increased, at the same time the melting temperature of the electrolytic bath can be reduced to about 750 to 950° C. and therefore the electrolysis can be effected smoothly at a temperature about 100 to 250° C. lower than in the conventional method.

Aluminum-sodium borofluoride is, as far as I know, first manufactured by me. Aluminum-sodium borofluoride is so stable as not to decompose even at a considerably high temperature. It melts completely at a comparatively low temperature of about 680 to 720° C. The solubility of alumina in aluminum-sodium borofluoride is high. I have found that 30 parts of alumina can be completely dissolved and melted in 100 parts of said borofluoride at about 720° C.

The manufacture of said borofluoride is not the purpose of the present invention and therefore details thereof are omitted. In general, said borofluoride is prepared as follows:

A solution of sodium aluminate or a mixed solution of sodium aluminate and sodium hydroxide

( $\text{AlNaO}_2$ — $\text{NaOH}$  or  $2\text{AlNaO}_2\text{—NaOH}$ )

is added to fluoboric acid. The reaction proceeds as shown in the following formulas and the aluminum-sodium borofluoride is formed as a white precipitate, said precipitate being then fractionated and dried:

- (1)  $3\text{HBF}_4 + \text{AlNaO}_2\text{—NaOH} \rightarrow \text{AlOBF}_4\text{—}2\text{NaBF}_4 + 2\text{H}_2\text{O}$
- (2)  $2\text{HBF}_4 + \text{AlNaO}_2 \rightarrow \text{AlOBF}_4\text{—NaBF}_4 + \text{H}_2\text{O}$
- (3)  $3\text{HBF}_4 + 2\text{AlNaO}_2\text{—NaOH} \rightarrow \text{Al}_2\text{Na}_3\text{O}_3(\text{BF}_4)_3 + 2\text{H}_2\text{O}$

For example, 1000 cc. of 1 mole solution of sodium aluminate combined with caustic soda ( $2\text{AlNaO}_2\text{—NaOH}$ ) were gradually added with stirring to 650 cc. of 33.5%

fluoboric acid solution. The reaction proceeded and difficultly soluble aluminum-sodium borofluoride was formed as a white precipitate. The whole was allowed to stand for one day and night to complete the reaction. The precipitate was then filtered, dried at 110° C., and was further roasted at 550 to 600° C. for 3 hours. By this way, 430 grams of the borofluoride having a melting point of 680 to 720° C. were obtained.

In carrying out the method of the present invention, in general, if the amount of sodium borofluoride and/or aluminum-sodium borofluoride relative to cryolite is increased, the melting temperature will be reduced while the solubility of alumina will be increased. However, the use of excess amount of sodium borofluoride and/or aluminum-sodium borofluoride is undesirable because it tends to cause the so-called anode effect in the electrolysis, to make the electrolysis difficult and to corrode the electrolytic cell and electrodes. For example, when a mixture of 100 grams of aluminum-sodium borofluoride, 100 grams of cryolite and 100 grams of alumina is heated in an electric furnace, it completely melts at a low temperature, namely 710° C. However, for the above mentioned reasons, this composition is not satisfactory as an electrolytic bath. On the other hand, when the amount of the use of sodium borofluoride and/or aluminum-sodium borofluoride is too small, satisfactory reduction of the melting temperature and increase in the solubility of alumina will not be attained.

I have found that the composition of 15 to 30% by weight of alumina, 50 to 80% by weight of cryolite and 5 to 20% by weight of sodium borofluoride and/or aluminum-sodium borofluoride is satisfactory in practice. That is to say, a mixture having the composition within this range completely melts at about 750 to 900° C. and its electrolysis proceeds smoothly and efficiently.

The melting and electrolysis operations and equipments to be used therefor are nothing particularly different from those in the existing methods. For example, an electrolytic bath mixture having the composition within the above mentioned range is put into an electrolytic cell which may be a crucible made of graphite and constitutes a cathode in case of electrolysis and is fused by a proper heating means such as electric furnace. Any known anode such as a graphite electrode is immersed in said fused electrolyte and the electric current is fed thereto for electrolysis. As the electrolysis proceeds, sodium borofluoride or aluminum-sodium borofluoride will be decomposed and lost little by little. Therefore, particularly when the electrolysis is carried out on a continuous basis a suitable amount of the compound must be properly added so that the electrolytic bath may maintain substantially the above mentioned range of composition. Similarly, aluminum fluoride in cryolite is decomposed and there is formed or separated sodium fluoride, which is accumulated as the electrolysis proceeds. Therefore, it is necessary to suitably add aluminum fluoride from time to time to reproduce cryolite and to keep the composition within the range mentioned.

Some examples of the present invention are given below for a more complete understanding of the invention. However, the invention is not to be limited to these examples.

### Example 1

A mixture of 203 grams of alumina, 172 grams of aluminum-sodium borofluoride and 625 grams of cryolite as an electrolyte was charged into a crucible which is made of graphite and is about 10 cm. in inside diameter and about 13 cm. in depth. Heat is applied thereto by means of an electric furnace and the mixture melted at 840 to 880° C. and came to maintain desired fluidity. A bar-shaped graphite anode of about 2 cm. in diameter

## 3

was immersed in the fused electrolyte in said electrolytic cell which is to constitute a cathode and the electric current was turned on to place the cell in electrolysis operation. The electrolysis proceeded under said temperature. The voltage ranged from 11 to 13 volts and the current density at the anode was 0.8 ampere/cm.<sup>2</sup>. About 6 hours later, deposition of about 51 grams aluminum was recognized in the bottom of the crucible.

## Example 2

A mixture of 153 grams of alumina, 129 grams of aluminum-sodium borofluoride and 718 grams of cryolite was put into a crucible (electrolytic cell) similar to that of Example 1 and was heated by an electric furnace. The mixture completely melted at 810 to 840° C. and came to maintain the desired fluidity. The electrolysis proceeded at the voltage of 10 to 13 volts and the current density (at the anode) of 0.7 ampere/cm.<sup>2</sup> for 7 hours in the same manner as in Example 1. About 56 grams of aluminum were deposited thereby.

## Example 3

A mixture of 152 grams of powdered alumina, 42 grams of aluminum-sodium borofluoride and 806 grams of cryolite was put into a crucible (electrolytic cell) similar to that of Example 1 and was heated by an electric furnace. The mixture completely melted at 860 to 890° C. and came to maintain the desired fluidity. When the electrolysis was proceeded at the voltage of 10 to 14 volts and the current density (at the anode) of 0.7 ampere/cm.<sup>2</sup> in the same manner as in Example 1, deposition of about 53 grams aluminum was recognized in 6.5 hours.

## Example 4

A mixture of 150 grams of powdered alumina, 150 grams of aluminum-sodium borofluoride and 700 grams of cryolite was heated in an electrolytic cell similarly to the preceding examples. The mixture completely melted at 760-800° C. and came to maintain the desired fluidity. The electrolysis proceeded under substantially the same condition as in Example 3 and deposition of about 62 grams of aluminum was recognized in 7.5 hours.

## Example 5

A mixture of 300 grams of powdered alumina, 90 grams of aluminum-sodium borofluoride and 610 grams of cryolite was put into an electrolytic cell similar to that of Example 1 and was heated by an electric furnace. The mixture completely melted at 890 to 910° C. and came to maintain the desired fluidity. The electrolysis proceeded at the voltage ranging from 11 to 13 volts and the current density (at the anode) of 0.7 ampere/cm.<sup>2</sup> in the same way as in Example 1 and after 6 hours about 48 grams of aluminum were deposited.

## Example 6

A mixture of 180 grams of powdered alumina, 190 grams of sodium borofluoride and 630 grams of cryolite was heated in an electrolytic cell similar to that of Ex-

## 4

ample 1. The mixture melted completely at 830 to 880° C. and came to maintain the desired fluidity. The electrolysis proceeded at the voltage ranging from 11 to 14 volts and the current density (at the anode) of 0.8 ampere/cm.<sup>2</sup> in the same manner as in Example 1 and after 6 hours deposition of about 45 grams of aluminum was recognized.

## Example 7

A mixture of 150 grams of powdered alumina, 140 grams of sodium boro-fluoride and 710 grams of cryolite was put into an electrolytic cell similar to that of Example 1 and was heated by an electric furnace. The mixture completely melted at 820 to 860° C. and came to maintain the desired fluidity. The electrolysis proceeded at the voltage ranging from 11 to 13 volts and the current density (at the anode) of 0.7 ampere/cm.<sup>2</sup> in the same way as in Example 1 and after 8 hours about 68 grams of aluminum were deposited.

It will be noted that the voltage in the above examples is somewhat higher than in the conventional method. However, this is caused by the fact that these specific examples are made on a small scale so that there are comparatively high contact resistance and other resistances. There will be no substantial difference of voltage if carried out on a large scale.

The capacity of the graphite crucible or electrolytic cell used in the above examples is small and accordingly temperature drop due to radiant heat loss is comparatively large. Therefore, in these examples, the electric current must be passed to the electric furnace at proper time in the electrolysis operation to maintain the desired fluidity. However, there would be no such necessity in case the electrolysis is carried out on a large scale because once the mixture is melted the temperature and fluidity can be maintained satisfactorily by the joule heat produced in the course of the electrolysis.

## I claim:

1. A method of preparing aluminum by electrolysis which comprises electrolyzing at a temperature from 750 to 950° C. a fused electrolyte consisting of 15 to 20% by weight of alumina, 60 to 80% by weight of cryolite and 5 to 20% by weight of a substance selected from the group consisting of sodium borofluoride, aluminum-sodium borofluoride and their mixture.

2. A method of preparing aluminum by electrolysis which comprises electrolyzing a fused electrolyte consisting of 15 to 20% by weight of alumina, 60 to 80% by weight of cryolite and 5 to 20% by weight of a substance selected from the group consisting of sodium borofluoride, aluminum-sodium borofluoride and their mixture.

## References Cited in the file of this patent

## UNITED STATES PATENTS

244,234 Higgs ----- July 12, 1881

## FOREIGN PATENTS

648,337 Great Britain ----- Jan. 3, 1951